

## UNITED STATES PATENT OFFICE

2,220,290

## RESINOUS MATERIAL

Alexander N. Sachanen and Pharez G. Waldo,  
Woodbury, N. J., assignors to Socony-Vacuum  
Oil Company, Incorporated, New York, N. Y., a  
corporation of New York

No Drawing. Application January 12, 1938,  
Serial No. 184,596

2 Claims. (Cl. 260—67)

This invention relates to the production of materials of a resinous nature. In particular the invention is concerned with the production of oil soluble resins from petroleum products.

5 Heretofore formolite resinous compositions have been produced by the action of formaldehyde on petroleum distillates and crude oils in the presence of sulphuric acid. These condensation products produced in the past, the so-called 10 formolites, are, however, oil insoluble resins, lacking the property of being easily molded and form brittle resins.

It is an object of this invention to provide a method for producing resinous materials from 15 solvent tars. A more specific object of the invention is to produce resinous materials from solvent tars comprising oil soluble resins. Other objects will, in part, be obvious and will in part appear hereinafter.

20 Contrary to the prior processes which produced only oil insoluble formolite resins from petroleum products, our invention is based upon the discovery that oil soluble resins may be produced in substantial amounts by treating solvent tars under proper conditions with formaldehyde or 25 suitable derivatives thereof. The resinous reaction product obtained contains in addition to oil soluble resins some oil insoluble formolites and unreacted oil. These three components of the 30 resinous product are usually present in approximately equal percentages but may be easily separated by means of solvent extraction and distillation.

35 Solvent tar is the well known rejected product obtained from the solvent refining of lubricant oils. In solvent refining a lubricating oil, a lubricating fraction of petroleum is contacted with a solvent capable of exerting selective solvent 40 properties upon the various constituents thereof for the purpose of separating the raw stock into two fractions. The raffinate or refined stock is a product of more highly paraffinic nature, more 45 stable, of higher viscosity index and a better lubricant. The solvent tar or discarded stock is more highly naphthenic and aromatic and of much lower viscosity index. As is well known, solvent tars vary in the amount of aromatic constituents which they contain. The aromaticity

of the tars varies according to the crude oil from which the petroleum fraction is derived to make the solvent tar. Thus, a solvent tar produced by refining a Coastal or a Mid-Continent oil is usually more highly aromatic than a solvent tar produced by refining a Pennsylvania oil. 5

In the practice of our invention we may employ any solvent tar which contains aromatic constituents; however, better results are obtained by use of solvent tars containing relatively high 10 percentages of aromatic constituents. Accordingly, for our purpose, we prefer to use solvent tars of the class which contain at least 65% of aromatic constituents (as measured by absorption with strong sulphuric acid), and especially 15 suitable are the solvent tars containing at least 75% of aromatic constituents, such as a furfural solvent tar obtained from the treatment of distillates from Mirando crude. Other solvent tars which may be mentioned merely by way of example as suitable tars for the practice of our 20 invention are the solvent tars obtained in the refining of distillates from East Texas crude and Rodessa crude. It is to be clearly understood, however, that the invention is not limited to the 25 use of the specific tars mentioned since solvent tars in general containing aromatic compounds may be used.

In place of formaldehyde various derivatives 30 thereof may be employed as the resinifying agent, such as paraformaldehyde and hexamethylene-tetramine. In view of the fact that all of these compounds have formaldehyde as a basis, for convenience they will be referred to hereinafter 35 in the specification and claims as formaldehyde resinifying agents.

In accordance with our invention, a suitable 40 solvent tar is mixed with a formaldehyde resinifying agent and reacted in the presence of an acid catalyst, such as sulphuric acid. A resinous material is formed containing oil soluble resins, oil insoluble formolites and unreacted oil. The resinous material thus formed is separated from the excess solution and extracted with any suitable 45 solvent such as petroleum ether or other suitable petroleum fraction, benzene, etc. After the extraction, the solvent extract which contains the oil soluble resins and unreacted oil, is 50

evaporated to remove the solvent and then distilled in vacuo to remove the unreacted oil. The yields of oil insoluble resins, oil soluble resins, and distillate oil are usually approximately equal, that is, about 30 to 35% of the amount of tar for each product.

While it is preferred to use sulphuric acid as the catalyst, the invention is not limited thereto, but mineral acids in general having a similar strength, such as hydrochloric, etc. may be used to give the desired acidity. After the completion of the reaction, water or acetic acid may be added to dilute the reaction mixture so as to aid in separation and removal of the sulphuric acid.

The oil soluble resins produced by our process are solid at normal temperature and on heating they are gradually liquified. Their color is dark red with a green fluorescence. Further, these resins are completely miscible with all oil products and when dissolved in oils they increase the viscosity of the oil. It has been found that these oil soluble resins also can be used for varnishes and other coatings and can be admixed with other resins to increase the plasticity of the resultant product.

While the oil insoluble resins may be used as such for certain purposes, they also can be admixed with other resins and used in various arts, for example molding.

The distillate oil obtained from our process can be used as a highly refined lubricating oil where a high viscosity index is not necessary. The viscosity index of these distillates usually does not exceed 0-20.

The invention will be further illustrated by the following examples. However, it is to be understood that the invention is in no way limited thereto.

*Example 1.*—One part of solvent tar (containing more than about 75 to 80% aromatic hydrocarbons) is mixed with approximately 10% by weight of paraformaldehyde, and while stirred continuously reacted for a period of about one hour in the presence of one part by volume of sulphuric acid (92%). Instead of paraformaldehyde, aqueous formaldehyde (30%) may be used in the amount of one volume with respect to the solvent tar. The resinous material produced is separated from the aqueous solution of sulphuric acid and excess formaldehyde, washed, dried and then extracted with petroleum ether. The petroleum ether extract containing the oil soluble resins and unreacted oil is then evaporated to remove the ether and distilled in vacuo to remove the oil. The total yield of raw formolites (oil insoluble formolites, oil soluble resins and unreacted oil) is about 100% based on the amount of tar used or slightly more. The yield

of oil soluble resins is about 35% of the amount of solvent tar and the yield of oil insoluble resin is similar.

#### Example 2

|                                                                           |     |    |
|---------------------------------------------------------------------------|-----|----|
| Furfural tar (from the treatment of distillates from Mirando crude) _____ | gr. | 50 |
| Paraformaldehyde _____                                                    | gr. | 5  |
| Glacial acetic acid _____                                                 | cc. | 50 |
| Sulphuric acid (94%) added slowly _____                                   | cc. | 50 |

5

10

The mixture is stirred for one-half hour then diluted with water, filtered, washed, dried and extracted with petroleum ether. Petroleum ether extract is evaporated to remove petroleum ether, and the residue is distilled in vacuo. The yields of the products are as follows:

|                          |     |    |
|--------------------------|-----|----|
| Formolites _____         | gr. | 15 |
| Oil soluble resins _____ | gr. | 27 |
| Distillate oil _____     | gr. | 10 |

20

#### Example 3

|                            |     |    |
|----------------------------|-----|----|
| Furfural tar _____         | gr. | 50 |
| Paraformaldehyde _____     | gr. | 5  |
| Sulphuric acid (80%) _____ | cc. | 50 |

25

The mixture is stirred for one half hour. The subsequent operations are the same as in Example 2. The yields of the products are as follows:

|                          |     |    |
|--------------------------|-----|----|
| Formolites _____         | gr. | 15 |
| Oil soluble resins _____ | gr. | 13 |
| Distillate oil _____     | gr. | 22 |

30

Since certain changes may be made in the invention without departing from the scope thereof, it is intended that all matter contained in the above description shall be interpreted as illustrative and not in a limiting sense.

35

We claim:

1. The method of preparing an oil soluble resinous material which comprises reacting a petroleum solvent tar containing at least 65% of aromatic constituents with approximately 10% by weight of a formaldehyde resinifying agent in the presence of a strong mineral acid catalyst from the group consisting of sulphuric acid and hydrochloric acid to form a resinous product comprising oil soluble resins, oil insoluble resins and unreacted oil, solvent extracting the resinous product to obtain a solvent extract containing oil soluble resins and unreacted oil, and subjecting the solvent extract to distillation to remove the solvent and unreacted oil thereby leaving the oil soluble resins as residue.

2. The oil soluble resin product prepared in accordance with the method of claim 1.

ALEXANDER N. SACHANEN.  
PHAREZ G. WALDO.

40

45

50

55